

## 1

2,820,745

PROCESS FOR ELECTROWINNING TITANIUM  
OR ITS CONGENERS

Foord von Bichowsky, Wilmington, Del.

No Drawing. Application January 12, 1953  
Serial No. 330,917

4 Claims. (Cl. 204—14)

This invention relates to a new and improved process for the obtaining of titanium and/or its congeners by electrolytic means.

Attempts to electrowin the metals of the fourth group of the periodic table of the elements and specifically to recover pure, titanium, zirconium or hafnium from aqueous solutions or from melts containing their compounds have resulted either in the deposition of very thin films or in the formation of a metal so dispersed within the melt that its recovery therefrom was very difficult.

Work also has been done toward plating out the metals of the fourth group from non-aqueous solutions of their halogen compounds. In those experiments the metals were used mainly in the form of their quadrivalent salts, for example, the readily available titanium or zirconium tetrachlorides, but because of the great chemical activity of such compounds the organic solvents employed, which were mostly of an alcohol or glycol type, probably reversibly reacted with those salts in accordance with the following typical equation:



and so, perhaps because of the linkage of titanium to oxygen in the resulting titanium ethylate, an oxygen free titanium could not be recovered from an alcoholic solution of that compound.

In order to overcome any such harmful chemical activity, of the tetrahalides of the metals of the fourth group of the periodic table of the elements, it occurred to me to study the use of certain double halogen or addition compounds of the above cited group of elements and as a result of that study and its extensions I made the discovery that the metals of the fourth group of the periodic table, when in solution, as their double halogen salts, in substantially non-aqueous solvents and while under oxidizing conditions, could be recovered therefrom in a commercially pure form when the conditions were so adjusted that the discharge potentials of the cations in the solvent were appreciably different.

The present invention thus covers the electrowinning of titanium and its congeners by the employment of a non-aqueous electrolyte, liquid at usual temperatures, which contains halogen salts of the metals of the fourth group, for example, titanium tetrachloride, associated with halogen salts of other metals and under oxidizing conditions.

The double halogen compounds of the fourth group of metals, in which the metal apparently has the coordination number 6 since it actuates 4 main valences and 2 minor valences, are represented by the salts, for example, of hexachlorotitanic acid.

That acid and its potassium and ammonium salts, as well as the sodium salt of the corresponding zirconium compound, are described in the literature and their preparation, for example, by salting out with hydrochloric acid or by reaction of the constituents, with and without pressure, is well known. I have also prepared those titanium compounds by reacting either hydrogen chloride or am-

## 2

monium chloride or potassium chloride, in an essentially non-aqueous solvent (i. e. one that contains no more H<sub>2</sub>O than is present in the commercial product) with titanium tetrachloride, either in concentrated form or diluted with, for example, carbon tetrachloride, in the cold. By that same general procedure I have interacted other metallic salts, in approximately the stoichiometrical amounts, with titanium tetrachloride or zirconium tetrachloride. Of the other metallic salts with which I have 10 experimented I will mention here only the chlorides of iron, copper, nickel, mercury, lithium, cadmium and lead but by following the above outlined technique the complexes of the metals of the fourth group of the periodic table may be formed either alone or intermixed with one 15 another or with the salts of other elements in various proportions and at various concentrations.

As usable solvents, for such metalloc-complexes or addition compounds of hexavalent titanium or its congeners and in which an electrolysis may be carried out under oxidizing conditions, I mention here the ternary compounds: 20 ethylene glycol, propylene glycol, glycerine, methanol, butanol, ethanol, propanol, ethyl ether, glycollic acid and/or other essentially anhydrous liquids fluid at room temperature which will conduct the electric current under the conditions of this invention.

In the process of the present invention the metal of the fourth group of the periodic system, when present as a complex of hexavalent titanium, or its congeners, with a chloride of another metal and while in a substantially 30 anhydrous solvent, appears to go directly from its high valence state down to that of the metal. In order to maintain that state of high valence an oxidizing agent, i. e. one that increases the positive valence of an element, is employed.

35 In theory any oxidizing agent; either gaseous, liquid or solid or combinations thereof, might be used to accomplish the above aim. In practice, however, it is found that not all oxidizing agents are equally advantageous because in certain cases some may be too active 40 and others too sluggish. Of the oxidizing agents tested in connection with this invention and in most cases with good results there may be mentioned gaseous or atmospheric oxygen or chlorine which latter may be generated in situ or added to the electrolyte. Of the solid oxidants, 45 ammonium persulfate, calcium hypochlorite, the normally insoluble higher oxides of lead or manganese or in special cases such compounds of copper or of iron as contain available oxygen may be cited. Barium peroxide also may be used but in that event the electrolyte should contain some free acid such as gaseous HCl or even HNO<sub>3</sub> in order to keep the pH of the solution on the acid side. Of the liquid oxidants one may use strong hydrogen peroxide or a concentrated solution of sodium hypochlorite or even nitric acid provided that they do not 55 react in a deleterious manner with the electrolyte.

In carrying out an electrolysis of a halogen complex of a metal of the fourth group, while in a solution in one or more of the useful solvents in substantially non-aqueous state, a simple cell may be used. There also may 60 be employed a cell which has partitions or diaphragms and in which the electrolyte either is stationary or is circulated within the separate compartments or else the application of circulation may be utilized in a cell of the simple type.

65 The cathode in the chosen cell may be of mercury, lead, copper, cadmium, titanium or zirconium or hafnium or of any satisfactory material or alloy, and it may be fixed or rotatable. For most purposes I prefer to use titanium or zirconium as a cathode and while, for example, mercury has a high hydrogen overvoltage it also has a tendency to form insoluble compounds such as mercurous chloride which can contaminate the deposit

and in addition mercury does not appear to wet titanium nor amalgamate therewith.

The anode may be of either a permanent or soluble type. Of the former I mention graphite and of the latter either impure or scrap titanium metal and its alloys or else a non-metallic substance, such as the active form of titanium nitride as mentioned in U. S. Patent No. 1,783,684, may be employed. In some cases and with non-aqueous solvents it may be desirable to carry out the electrolysis at a temperature above that of room provided that the solvent is not appreciably harmed thereby.

Having now, in general, outlined the method of this invention I will illustrate it by a specific example:

To 189 g. of very pure  $TiCl_4$  (1 mol) and which has been cooled nearly to freezing (ca. -25° C.) there is added 15 one mole of dried anhydrous  $CuCl_2$  (134 g.) and the mixture is further cooled while stirring until the brown mush of  $CuCl_2 \cdot TiCl_4$  solidifies or freezes whereupon there is added thereto 1 liter of commercially anhydrous methanol, precooled to below 0° C. The brown 20 sediment or mass of the addition complex gradually dissolves as it thaws and when all is in solution the resulting greenish liquid is divided into two portions. To the part to be used as the catholyte there is added about 20 g. of ammonium persulfate and the gently stirred suspension 25 is electrolyzed using a compartmented cell. The untreated remainder of the greenish liquid is placed in the anode compartment. When using the above arrangement and with a graphite anode and a sheet of titanium as the cathode the resulting titanium metal is deposited thereon, 30 at a current density of about 150 amps./ft.<sup>2</sup> as a more or less spongy mass.

By means of various changes in the current density and through the use of other oxidizing means or solvents the titanium may be obtained in different particle shapes 35 and sizes. In most cases it is desirable to recover the metal with a minimum of occluded electrolyte as that facilitates its washing and working up.

In like manner zirconium or hafnium may be elec-  
trowon from a solution of their double salts in glycol or 40

in alcohol by using, for example, calcium hypochlorite as an oxidizing agent.

Now having described my invention what I claim is:

1. Process for the electrolytic production of titanium which comprises passing an electrolyzing current from an anode through an anhydrous anolyte which consists essentially of a solution of  $CuCl_2 \cdot TiCl_4$  complex dissolved in an organic solvent selected from the group consisting of ethylene glycol, propylene glycol, glycerine, methanol, ethanol, propanol, ethyl ether and glycolic acid, to a cathode through a catholyte consisting essentially of a solution of said complex and sufficient ammonium persulfate to maintain the titanium in the tetravalent state in one of said solvents.

2. The process of claim 1, wherein the selected organic solvent is methanol.

3. Process for the electrolytic production of titanium which comprises passing an electrolyzing current from an anode through an anhydrous anolyte which consists essentially of  $CuCl_2 \cdot TiCl_4$  complex dissolved in methanol to a cathode through a catholyte consisting essentially of said solution of said complex and sufficient ammonium persulfate to maintain the titanium in the tetravalent state in said catholyte.

4. Process of claim 3, in which the anode is of graphite and the cathode is of titanium where the current density of the electrolyzing current is essentially 150 amps./ft.<sup>2</sup>.

#### References Cited in the file of this patent

#### UNITED STATES PATENTS

1,922,847 Grenagle Aug. 15, 1933  
2,510,128 Miner et al. June 6, 1950

#### OTHER REFERENCES

"Journal of The Electrochemical Society," vol. 98 (1951), pages 33C-35C, paper by Holt.  
Wright Air Development Center Technical Report #52-232, "Electrodeposition of Titanium from Aqueous Systems," December 1952.